

Nov. 12, 1940.

E. WHITWORTH ET AL

2,221,391

MANUFACTURE OF DOUBLE BASE PROPELLENT POWDERS

Filed July 28, 1939



*Thomas Thomson*  
*Edward Whitworth* INVENTORS

BY *Thos. A. Wilson*

ATTORNEY

## UNITED STATES PATENT OFFICE

2,221,391

MANUFACTURE OF DOUBLE BASE  
PROPELLENT POWDERS

Edward Whitworth, Saltcoats, and Thomas Thomson, Kilmarnock, Scotland, assignors to Imperial Chemical Industries Limited, a corporation of Great Britain

Application July 28, 1939, Serial No. 286,970  
In Great Britain August 2, 1938

5 Claims. (Cl. 52—13)

The present invention relates to the manufacture of double-base propellant powders; that is to say, propellant powders in which the active base comprises both nitrocellulose and nitroglycerine.

In the manufacture of certain propellant powders, nitrocellulose, in the form of nitrated comminuted paper board or the like, has been directly treated with nitroglycerine; these powders however retain a fibrous structure, and are not free-flowing. In the manufacture of non-fibrous free-flowing granular double-base propellant powders it has hitherto been necessary to gelatinise the fibrous nitrocellulose by a volatile or non-volatile nitrocellulose solvent, with or without nitroglycerine; the grains being formed after gelatinisation irrespective of the original degree of subdivision of the fibrous nitrocellulose.

This invention has as an object to devise a new method of manufacturing granular double-base propellant powders. A further object is to devise such a method which will provide a non-fibrous free-flowing granular powder with greater simplicity and economy than by known methods. Further objects will appear hereinafter. These objects are accomplished by the following invention.

We have found that we can achieve these objects by employing nitrocellulose in the form of a product obtained by the nitration and comminution, in either order, of regenerated-cellulose sheet material, and treating the product with nitroglycerine in the presence of a volatile medium that is a non-solvent for nitrocellulose. The non-fibrous nature of regenerated-cellulose sheet material and its nitration product renders it possible to effect the comminution of these materials to a size suitable for powder-grain formation (without destruction of the lamellar form of the particles); and the sheet material may be, if desired, partly or wholly comminuted while in the water-wet state by mechanical means, such, for instance, as beating or pulping machines. The comminution may be carried out partly or wholly before or after the nitration of the regenerated cellulose.

The comminuted nitrated regenerated-cellulose sheet material may, for instance, be produced by nitration of deglycerinated scrap commercial regenerated-cellulose sheet of about 0.001 in. in thickness. Such scrap material can be obtained for instance from the waste left when sheets of regenerated cellulose material are cut to size. A suitable method for the production of nitrated regenerated-cellulose sheet material for the purposes of the present invention consists in com-

minuting the waste commercial regenerated-cellulose sheet into the form of small crumpled pieces of single thicknesses and washing repeatedly with water, for instance at a temperature of about 40° C.—45° C., to remove the polyhydric alcohol employed as softening agent, and to float off any lacquer that may have been applied to the surface of the sheet. The product thus freed from foreign constituents is centrifuged, dried, and nitrated, advantageously at a temperature of 10 40° C.—60° C. with from 20—45 parts by weight of a nitrating acid containing at least 16% of water, sulphuric acid in amounts up to 65% and from 19—30% nitric acid. The fragments of comminuted nitrated regenerated-cellulose sheet material may, for instance, be less than 1 mm. square.

Another suitable method for the production of comminuted regenerated cellulose sheet material is to comminute such sheet material of about 0.001 in. 20 thickness in a pulper to fragments of a size varying from about 0.01 in. square up to about 0.04 in. square.

The treatment of the comminuted nitrated product with nitroglycerine in a nitrocellulose 25 non-solvent volatile medium may be carried out with agitation in known manner; e. g. in aqueous suspension or by use as a vehicle of another liquid that does not dissolve nitrocellulose. Modifiers or other additional ingredients may be 30 introduced into the product either at the same time, or subsequently. During the treatment of the nitrated comminuted regenerated cellulose with the nitroglycerine, the particles may agglomerate to some extent; but powders of satisfactorily uniform grain size and excellent ballistic 35 properties can nevertheless be obtained in the manner described.

The invention is further illustrated but not limited by the following examples, in which the parts 40 are parts by weight, and which refer to the production of shotgun powders.

## Example 1

Scrap commercial regenerated cellulose material about 0.001 in. in thickness is comminuted in a pulper to fragments of a size varying from about 0.01—0.02 in. square up to about 0.04 in. square. The comminuted mass is washed with hot water at 45° C. to remove all soluble foreign 45 matter from the regenerated cellulose and to float off any insoluble lacquer or wax coating. The purified comminuted regenerated cellulose is centrifuged, dried, and nitrated at a temperature not exceeding 40° C. with 25 times its weight of a 50 55

nitrating acid containing 35.2% sulphuric acid, 50% nitric acid and 14.8% water, washed and stabilised.

100 lbs. of this nitrated regenerated cellulose 5 made from commercial material 0.001 in. thick in comminuted thin sheet form, are suspended in 300 lbs. water at 25° C. in a rotating copper pan. 10 40 lbs. nitroglycerine containing 5 lbs. diethyl phthalate are added gradually through a rose-spray, and mixing is continued for 1 hour.

The pan is then discharged and the impregnated powder is steeped for 24 hours at 60° C. in a solution containing, for every 100 lb. nitrated regenerated cellulose, 87 lb. barium nitrate and 15 21 lb. potassium nitrate dissolved in 56 gallons of water. At the end of this time the powder is removed and drained. It is sieved while still wet through an 18 mesh sieve to break up any undesirably large aggregates and is then transferred 20 to a drying stove at 43° C. for a period of 24 hours.

The dry powder is finally surface graphited with 1% graphite, sifted and blended according to standard procedure.

25 *Example 2*

100 lb. nitrated regenerated cellulose as used in the process of Example 1, and 8 lb. finely ground 2:4 dinitrotoluene are mixed in a rotating copper 30 pan for 5 minutes, and 300 lb. water are added at 25° C. 40 lb. nitroglycerine are added gradually through a rose-spray, and mixing is continued for a period of 1 hour.

The subsequent procedure is identical with 35 that described in Example 1.

As stated above, we prefer to use regenerated cellulose sheet of about 0.001 in. thickness, but we could get good results with thicknesses which lie between 0.0005 and 0.01 in. We prefer to 40 break this up into lamellae of a size between 0.0004 and 0.0025 sq. in. but sizes between 0.000025 and 0.0156 sq. in. are also useful provided that the size is chosen in accordance with the thickness of the sheet so that the general lamellar 45 shape is retained. "Dust" is undesirable and is sieved out from the nitrated product.

The finished grain should not exceed 0.125 in. in diameter, and we prefer to use grains which will pass through an 18 mesh sieve which has 50 apertures about 0.033 in. square.

While the product of our invention has been described in detail in the foregoing, it is believed that the nature of this product will be appreciated more fully from the illustration of the same in the accompanying drawing which shows 5 clearly the characteristic form of the same comprising rounded masses including nitroglycerin and aggregations of lamellar fragments of nitrated regenerated cellulose sheet material. The size of these particular grains is indicated by 10 the fact that the illustration represents a magnification of 20 diameters.

As many apparently widely different embodiments of this invention may be made without departing from the spirit and scope thereof, it is 15 to be understood that the invention is not limited to the specific embodiments thereof except as defined in the appended claims.

We claim:

1. A process for the manufacture of a double- 20 base propellant powder that includes the step of agitating comminuted and nitrated regenerated-cellulose sheet material with nitroglycerine in presence of a volatile liquid that does not dissolve nitrocellulose.

2. A double-base propellant powder comprising 25 rounded masses including nitroglycerin and aggregations of lamellar fragments of nitrated regenerated-cellulose sheet material.

3. A double-base propellant powder comprising 30 rounded masses including nitroglycerin and aggregations of lamellar fragments of nitrated regenerated-cellulose sheet material, the said rounded masses being less than 0.125 in. in 35 diameter.

4. A double-base propellant powder comprising 40 rounded masses including nitroglycerin and aggregations of lamellar fragments of nitrated regenerated-cellulose sheet material, the said lamellar fragments having a thickness between 0.0005 and 0.01 inch and a size between 0.000025 and 0.0156 square inch.

5. A double-base propellant powder as claimed 45 in claim 2 in which the size of the lamellae lies between 0.0004 and 0.0025 square inch.

EDWARD WHITWORTH.  
THOMAS THOMSON.